

## UNITED STATES PATENT OFFICE

2,321,517

## LUBRICANT COMPOSITION

Raphael Rosen, Elizabeth, N. J., assignor to  
 Standard Oil Development Company, a corpora-  
 tion of Delaware

No Drawing. Application January 2, 1941,  
 Serial No. 372,839

1 Claim. (Cl. 252—34)

The present invention relates to an improvement in lubricants and similar oils, as well as other hydrocarbon materials, especially in respect to resistance to decomposition at elevated temperatures and oxidizing conditions such as are encountered in internal combustion engines. The invention will be fully understood from the description which follows.

It has been found that mineral oil lubricants can be greatly improved with respect to their ability against decomposition, especially under heat and oxidizing conditions, by the addition thereto of small amounts of certain substances. In the present case, a new group of substances has been discovered which are particularly effective in reducing the oxidation of oils at the elevated temperatures encountered in internal combustion engines, i. e., at temperatures of 200° C. or higher. This group of substances comprises inorganic salts of quaternary ammonium bases. Such compounds are soluble in mineral oil to only a small extent when the nitrogen atom of the compound is attached to short hydrocarbon radicals. Greater solubility can be imparted to the compound by increasing the length of the aliphatic radicals and compounds with a total of at least 12 carbon atoms in all. The aliphatic radicals are most desired for the purpose of the present invention. Compounds that are insoluble may, however, be used by being dispersed in the oil or when dissolved by the aid of a mutual solvent.

In its broadest aspects, the preferred class of new addition agents includes the compounds having the formula:



Where R is a hydrocarbon radical, for example, alkyl, cycloalkyl, aryl or aralkyl radical, X is an inorganic acid radical, and m is an integer, one or less, chosen according to the valencies of the R groups to satisfy four bonds of the nitrogen atom. The various R groups may be similar or dissimilar. The radicals R may contain substituent atoms, for example, halogen, nitrogen, phosphorus, oxygen or sulfur, or substituent groups, for example, hydroxyl, aroxy, oxy, keto, amino or mercapto groups. The preferred compounds are those in which the R groups are alkyl groups. The most preferred compounds are those in which the total number of carbon atoms in all of the hydrocarbon radicals is at least 12 and preferably at least 16, if possible. The acid radical may be of any type inorganic acid radical, but the salts most pre-

ferred are the halides, phosphates, phosphites, thiophosphates, thiophosphites, cyanates and thiocyanates of the ammonium bases. It is desirable to select compounds which are soluble in lubricating oil to the extent of at least 0.5% at temperatures above 30° F. Typical examples of suitable compounds are tetra-n-butyl ammonium iodide, tetra-n-butyl ammonium bromide, octadecyltributyl ammonium iodide, benzyl octadecyl dimethyl ammonium chloride, octadecyl benzyl dimethyl ammonium chloride, cyclohexyl triisobutyl ammonium phosphite, phenyl tridecyl ammonium thiocyanate, triethanol octadecyl ammonium sulfite, methyl pyridonium sulfide and chloorethyl tributyl ammonium nitrate. In addition to the above, suitable examples include the nitrites, sulfites, hypophosphites, borates, stannates, arsenates, arsenites, chromates and chromites of various quaternary ammonium bases.

The new class of antioxidant compounds are advantageously added to the oils in concentrations ranging from 0.05 to 5%, but the quantity generally preferred is about 0.1 to about 1%.

In general, the base stock to be used in the preparation of the lubricants of the present invention may be any refined mineral lubricating oil, preferably having a viscosity from 40 to 150 seconds Saybolt at 210° F., and suitable base stocks include those of high paraffinic and high viscosity index, such as those which have a viscosity index of 100 or more, as well as low paraffin and low viscosity index oils. Base stocks comprising greases, fatty oils or synthetic oils may also be employed.

The addition agents of this invention do not have any detrimental effects on the physical character of the lubricating oil to which they are added, such as viscosity, gravity and flash point.

The new additives may be used as the sole blending agents, or they may be added with other ingredients, such as oiliness agents, film strength modifiers, pour depressants, thickeners, viscosity index improvers, detergents, sludge dispersers, solvents, dyes, and the like.

The compounds described above may be used as oxidation inhibitors and improving agents in similar concentrations in other lubricating oil products, such as lubricating greases and extreme pressure lubricants.

The value of the antioxidants of the present invention when used in lubricating oil blends has been determined by several standard tests, including the oxygen absorption test, the cone 55 test and the Sligh oxidation test.

The oxygen absorption test is carried out by bubbling a known amount of oxygen through 10 cc. of the lubricating oil maintained at 200° C. The oxygen is continuously recycled. At the end of succeeding 15 minute periods the amount of oxygen absorbed by the oil is measured. The results are given as the number of cubic centimeters of oxygen absorbed during each of these 15 minute periods.

The cone test, which is a means for determining the tendency of an oil to deposit solid material upon heated metallic surfaces, is carried out by slowly dropping oil to be tested over a heated metal cone having a circumferential groove milled out in a screw fashion on the periphery so as to allow a time of contact of about one minute between the heated metallic surfaces and the oil. A total volume of 60 cc. of oil is dropped from a dropping funnel during a period of two hours, the temperature of the cone being maintained at 250° C. The cone is then washed in naphtha to remove adhering oil and the total deposit determined by difference in weight.

The Sligh oxidation test is carried out by heating 10 grams of the oil, contained in a stoppered conical flask from which the air has been displaced by oxygen, at 200° C. in an oil bath for 2½ hours. The number of milligrams of asphaltenes formed, determined by a solution of the oil in precipitation naphtha and filtration through a Gooch crucible, is termed the Sligh number of the oil.

The value of the antioxidants of the present

invention as addition agents for lubricating oils may be illustrated by the following example.

*Example*

5 A refined mineral lubricating oil of S. A. E. 50 grade was blended, separately, with 0.2% of tetra-n-butyl ammonium iodide and 0.2% of tetra-n-butyl ammonium bromide, and the blends thus formed, as well as a blank sample of the base 10 oil, were submitted to the cone test, the oxygen absorption test and the Sligh oxidation test, these tests having been described above. The results are as follows:

| 15 | Oil or blend                                      | Cone rating | Oxygen absorption | Sligh oxidation No. |
|----|---------------------------------------------------|-------------|-------------------|---------------------|
| 20 | Base oil.....                                     | 50          | 103-213-107       | 5                   |
|    | Base oil+0.2% tetra-n-butyl ammonium iodide.....  | 40          | 14-20-62-85       | 3.9                 |
|    | Base oil+0.2% tetra-n-butyl ammonium bromide..... | 40          | 30-51-46-47       | .....               |

The present invention is not to be considered 25 as limited by the herein described example, which is given by way of illustration only, but it is to be limited solely by the terms of the following claim.

I claim:

30 A lubricant containing dissolved therein 0.05% to 5% of tetra-n-butyl ammonium iodide.

RAPHAEL ROSEN.